

Aug. 6, 1940.

**W. E. BAHLS**

2.210,699

## VACUUM TIGHT INSULATED LEAD-IN STRUCTURE

Filed Oct. 21, 1936

4 Sheets-Sheet 1



**WITNESSES:**

C. J. Weller.  
R. W. Bailey

INVENTOR

BY *F. W. Lyle.*  
ATTORNEY

Aug. 6, 1940.

W. E. BAHLS

2,210,699

VACUUM TIGHT INSULATED LEAD-IN STRUCTURE

Filed Oct. 21, 1936

4 Sheets-Sheet 2



Aug. 6, 1940.

W. E. BAHLS

2,210,699

VACUUM TIGHT INSULATED LEAD-IN STRUCTURE

Filed Oct. 21, 1936

4 Sheets-Sheet 3

Fig. 10.



Fig. 11.



Fig. 12.



Fig. 13.



Fig. 14.



WITNESSES:

C. J. Weller  
R. W. Bailey

INVENTOR  
Walter E. Bahls.  
BY F. W. Lyle.  
ATTORNEY

Aug. 6, 1940.

W. E. BAHLS

2,210,699

VACUUM TIGHT INSULATED LEAD-IN STRUCTURE

Filed Oct. 21, 1936

4 Sheets-Sheet 4

Fig. 15.



Fig. 16.



WITNESSES:

C. J. Welles  
R. W. Bailey

INVENTOR  
Walter E. Bahls.

BY  
F. W. Lyle.  
ATTORNEY

## UNITED STATES PATENT OFFICE

2,210,699

VACUUM-TIGHT INSULATED LEAD-IN  
STRUCTURE

Walter E. Bahls, Forest Hills, Pa., assignor to  
Westinghouse Electric & Manufacturing Company,  
East Pittsburgh, Pa., a corporation of  
Pennsylvania

Application October 21, 1936, Serial No. 106,798

6 Claims. (Cl. 250—27.5)

My invention relates to a vacuum-tight insulated lead-in construction and especially such construction applied to electron discharge devices.

5 An object of my invention is to provide a very strong vacuum-tight lead-in construction that will withstand a great difference of pressure on its opposite sides.

Another object of my invention is to provide 10 a lead-in construction for vacuum devices which will permit the utilization of much higher temperatures during the exhausting and degasifying of the parts.

Other objects and advantages of my invention 15 will become apparent from the following description and drawings, in which:

Figure 1 is a view through a hot cathode device incorporating my invention with the walls in cross section and the lead-in and interior parts in elevation.

20 Fig. 2 is a sectional view of a modification of Fig. 1.

Fig. 3 is a sectional view of a still further modification of Fig. 1.

25 Fig. 4 is a view through a mercury pool type of device incorporating my invention with the walls in cross section and the lead-in and interior parts in elevation.

Figs. 5, 6, 7 and 8 are modifications of the lead-in construction of Fig. 4.

30 Fig. 9 is a view principally in cross section of another mercury pool type of device incorporating further modifications of my invention.

Fig. 10 is a view principally in cross section of a lamp incorporating my invention.

35 Fig. 11 is a view mainly in cross section of a still further modification of the lead-in construction as applied to the mercury pool type of device of Fig. 4.

Figs. 12, 13 and 14 are still further modifications of the seal of Figs. 4 and 11; and,

40 Figs. 15 and 16 are curves illustrating the expansion of preferred materials utilized in the preceding seal construction.

45 In the prior art devices employing seals between lead-ins and metal containers, glass has been heretofore utilized. In such constructions, principally that of vacuum electron discharge tubes, it is necessary that the device be heat treated at a very high temperature in order to degasify the interior elements. An extensive portion of a glass wall cannot be utilized with such heat treatment because the glass will become molten and collapse. On the other hand, if not 50 much glass is used, there is apt to be a very short

distance between the lead-in and the metal wall of the container that will provide a leakage path with the accumulation of dirt and moisture.

It is an object of my invention to utilize a 5 ceramic material for the body of insulating material and to utilize a coating of glass to seal the ceramic material to the metal casing. I also contemplate using special forms by which the device will withstand pressure from within or without.

Figure 1 illustrates a particular type of discharge device utilizing my invention. This device has a container wall 10 of metal and preferably of an alloy of 24% to 30% nickel, 5% to 25% cobalt, less than 1% manganese and the remainder iron and known under the registered 10 mark "Kovar." The container wall is in the form of a tube with one end 11 closed and the open end having a flange 12 extending preferably outward. On this flange 11 is placed an annular ring 13 of ceramic material, preferably porcelain, 15 and having a certain desired number of openings 14 therethrough. These openings 14 have a tapered contour 15 preferably decreasing in diameter towards the inner portion of the device. The lead-in connection 16 is preferably formed 20 with a similar contour 17. The top portion is preferably closed with a plate 18 of metal 25 preferably similar to that of the container wall 10 and this plate has the desired tubulation 19 through which the device is exhausted. This 30 tubulation 19 can, of course, be at any other convenient portion of the device and it is understood that this tubulation, while it is not illustrated in the other figures, can be applied thereto. In assembling the device, the openings 14 35 are coated with a glaze or sealing material, preferably of glass and such glass is preferably of the boro silicate type of glass. This glass has a major percentage of silicon dioxide and also preferably has such silicon dioxide in an amount from 65% to 75%. This glass also preferably has less than 10% PbO, less than 6% Al<sub>2</sub>O<sub>3</sub> and 10% to 25% B<sub>2</sub>O<sub>3</sub>. The particular type of glass that I prefer to use has the following analysis:

|                                | Per cent |
|--------------------------------|----------|
| SiO <sub>2</sub>               | 67.3     |
| B <sub>2</sub> O <sub>3</sub>  | 24.6     |
| Al <sub>2</sub> O <sub>3</sub> | 1.73     |
| Na <sub>2</sub> O              | 4.6      |
| K <sub>2</sub> O               | .94      |
| As <sub>2</sub> O <sub>3</sub> | .50      |
|                                | .14      |

The surfaces 21 and 22 of the porcelain adjoining the metal portions 12 and 18 are also coated with this glass material. The lead-in 55

wires with their tapered contour are pushed into the tapered openings 14 and the interior structure assembled on their inner ends. Such interior structure may, for example, be the cathode 23, which may be of the directly heated type, and the grid structure 24. The device is then exposed to a high temperature at which the glass melts and seals the metal to the porcelain. The device is then evacuated. To facilitate the exhaust the device is heated to a high temperature and preferably to as high a temperature as the structure will withstand because the higher the temperature, the easier the gas will be evolved from the parts. Because of the arrangement of parts the device can be heated to the order of 700° C. or even above which temperature is above the melting point of the glass. Although the glass is softened, yet it will remain in place due to its thin film and very high viscosity. It will be noted that due to the tapered contour of the lead-in 16 and the opening 14 in the porcelain that a very firm seal is made therethrough and that the vacuum within the container will draw the lead-in tapered pin into a tighter seal in the opening. In other words, a greater pressure on the exterior of the device will only more firmly seal the tapered pin in the tapered opening in the porcelain material.

Also to facilitate exhaust by the cleaning up of oxides on the parts, I prefer to utilize an atmosphere of hydrogen about the device during part of the exhaust. At the high temperatures permitted by my arrangement the hydrogen will diffuse through the walls and reduce the oxides.

35 The glass, although utilized to seal the metal and porcelain, may also be used as a glaze to cover the exposed parts of the porcelain. Porcelain has a generally rough surface that would tend to retain dirt and moisture that would make a leakage path across its surface. Such dirt and moisture is not so apt to remain on a smooth glass surface. For this purpose any standard glazes may be utilized.

40 The parts disclosed in Fig. 1, as well as in the other figures, can be made self aligning and thus the need for a skilled glass blower will be eliminated.

Fig. 2 shows a somewhat similar construction utilizing somewhat the same container 10 with its flange 12. In place of the annular ring of Fig. 1, a plate or disc 30 of ceramic material which may be coated with a glass 31 is utilized. The lead-ins 32 preferably have the same tapered contour 33 but these are preferably sealed in tapered vertical openings 34 in the plate 30. The assembly of Fig. 2 is similar to that of Fig. 1.

In Fig. 3, the construction is still further modified in which a tapered disc or plate of porcelain 40 is utilized and is sealed in the tapered opening 41 of a metal plate 42 by means of a coating of glass 43 preferably similar to that previously described. The lead-ins 44 may have a very small bead or tapered portion 45 to be matched by a similar slightly tapered contour of the exterior portion of the openings 46. The construction of Fig. 3 is especially adaptable where the metal portion 42 sealed to the porcelain or ceramic material is rather expensive and it is desired to utilize some other cheaper metal, such as steel or iron, for the major portion 10 of the metal casing. Any suitable material can be used for portion 10 provided it is sufficiently non-porous and can be welded or otherwise made sufficiently vacuum tight to the portion 42.

75 Fig. 10 has a further modification of the in-

vention applied to a lamp in which a glass container 10 is sealed to a porcelain disc 50 at 51. The filament structure 52 has lead-ins 53 welded or copper sweated into pins 54. These pins 54 are of the preferred glass sealing metal of iron, nickel and cobalt described above. These pins have a tapered contour 55 that is sealed in tapered openings 56 in the disc 50, as described in connection with Fig. 1.

It will be noted that in Figs. 1, 2 and 3, the exterior casing 10 has been illustrated as that of an anode, although it is apparent that the tube structure might be modified to utilize it as one of the other electrodes. In the other figures illustrating the complete device, I have shown the exterior casing as making a connection to the cathode, which is disclosed as a mercury pool. In Fig. 4, for example, the metal container 60 has the mercury pool 69 forming the cathode therein. To this container 60 is welded a metal plate 61 preferably of the nickel cobalt iron alloy previously described, and having an outwardly extending tubular flange 62. If desired the flange part 62 only may be of this nickel cobalt iron alloy. This tubular flange 62 is sealed to an annular ring 63 of porcelain. This annular ring has preferably a slot 58 into which the edge of the flange 62 extends and which slot is filled with glass, preferably of the boro silicate type previously described for making a vacuum-tight seal between the metal 62 and the annular ring 63. A cup shaped cap 64 has preferably a downward extending flange 65 fitting into an upper annular slot 66 of the porcelain ring and sealed thereto by means of the aforementioned glaze. A lead-in 67 of any desired metal is welded to the inner side of the cup and at its inner end preferably supports an electrode such as the anode 68. An exterior conductor 69 can then be welded to the exterior surface of the cup to make contact therethrough to the interior electrode structure.

This type of device may have any one or a combination of auxiliary electrodes. One such type would be a make-alive 70 constructed of a high resistance material such as carborundum or boron carbide in contact with the mercury and supported by a conductor 71. This conductor 71 could have an exterior connection 72 connected to conductor 71 by a cap 73 sealed in a ceramic ring 74 similar to the supporting and connecting structure of the anode 68.

Fig. 5 illustrates a modification of the seal of Fig. 4. In Fig. 5, the flange 76 has preferably an outwardly tapered portion 77. The porcelain section 78 has a similar contour 79. The upper portion of the porcelain section also has a downwardly tapered opening 80 terminating in the flat portion 81 adjacent the central opening 82. The metal closing portion for this porcelain section has a corresponding taper 83 similar to 60 tapered opening 80 and also a flat area 84 to rest upon the flat area 81 and to close the central opening 82. The anode conductor 85 is welded to the under side of this metal closure and an exterior conductor 86 is welded to the upper side 65 of the metal closure 84. The metal portions are sealed to the porcelain by means of the glass glaze 87 previously described. It will be noted how the tapered portion of the porcelain at 79 and the tapered portion 77 of the metal casing will provide a very tight seal if a vacuum is maintained within the device and the exterior pressure will cause the porcelain to set more firmly on the tapered flange 77.

Fig. 6 illustrates a modification of the upper 75

portion of the device in Fig. 5, in which the metal portion 88 is tapered down and outwardly instead of upwardly as in Fig. 5. The flat portions 81 of Fig. 5 may be eliminated, as shown in Fig. 6.

Fig. 7 illustrates a very firm seal in which the ceramic portion 90 has an inwardly tapered portion 91 extending to a small diameter portion 92. Surrounding this ceramic portion is a tubular metal portion 93 extending inwardly at 94 to meet the tapered portion 91 at 95 and then extending in a contour at 96 similar to that of the porcelain until it forms an extending tubular portion 97 for the large diameter of the porcelain. A cap shaped metal closure member 98 seals the central opening of the porcelain containing the conductor 99. An exterior lead 100 is welded to the cap 98. In this construction, the cap 98 and the tubular member 93 may be of the nickel cobalt iron alloy previously described which will seal to the glass coating 101 of porcelain and other metal material may be used for the main portion of the metal container 102.

In case it is not desired to have the sealed lead-in construction extending from the exterior portion of the casing but to be placed mainly within the confines of the casing, a structure such as that illustrated in Fig. 8 may be utilized. In this case, a tube 105 is welded to the interior side of the casing 106 adjacent the opening 107 for the lead-in 108 therethrough. The inner end 109 of this tube is tapered and the porcelain section 110 has a similar tapered portion 111 that fits snugly adjoining the tapered portion 109. A sealing glass material 112 such as the boro silicate glass previously described seals the porcelain to the metal. The exterior lead-in 108 is welded to a cap 113 which may be similar to the caps previously described, such as that of Fig. 5, and this cap in turn has the anode conductor 114 welded to its inner surfaces.

The lead-in structures which have been previously described may be easily modified or combined to give a double or concentric type of lead. An example of such a lead for a pool type tube in which the starting electrode comes through the anode is disclosed in Fig. 9. The metal casing 120 containing the mercury pool 121 is illustrated in cross section. Preferably on the upper portion of this container is a metal tube 122 having a flange 123 sealed to and supporting a porcelain ring 124 similar to the porcelain rings of Figs. 5 and 6. A metal cap 125 preferably similar to the cap 88 of Fig. 6 is sealed to the porcelain ring 124. Instead of this cap closing the large opening 126 in the porcelain ring 124, it has an opening 127 centrally located therein and formed by a downwardly tapered flange 128. A smaller porcelain tube 129 is sealed to this flange 128 at its similar tapered portion 130. A cap 131 closes the central opening in this porcelain tube 129. This cap may be of any of the types previously described and as illustrated it is similar to that of Fig. 7. An exterior lead-in 132 is welded to the cap 131 and a conductor 133 is welded to the interior portion of the cap 131 and extends downwardly and has a make-alive 135 supported in position thereon to make contact with the mercury 121. Surrounding this make-alive lead-in construction is preferably an insulating quartz sleeve 134.

Welded to the interior side of the cap 125 is a tubular conductor 136 supporting on its inner end an anode 137 which, of necessity, has a hollow opening therethrough for the passage of the make-alive conductor and insulating sleeve. If

desired, the anode tubular support 138 may be likewise insulated by means of an insulating sleeve such as quartz 138 and an anode exterior lead 139 may be welded to the cap 125.

It is intended, of course, that the construction in Fig. 9 is illustrative of a preferred combination of the shapes of elements previous disclosed and that other specific shapes may be substituted in this combination.

Sometimes it is found desirable in the construction of metal tubes, for example, to assemble all the parts and then copper sweat all the vacuum joints. In a case of this sort, it is necessary to still have the leads come in through insulation. This type of assembly, however, presents a difficulty because of the decomposition of the glass glaze under the conditions for making the copper sweat joints. I have devised a structure in which the joints can be copper sweated and the parts cemented together with a high temperature cement or mechanically clamped. The structure is thus held rigidly in place while it is heated up to the temperature necessary to melt the copper or whatever metal may be necessary for the sweating process. After the sweating has been done, the glass may be put on to make the vacuum-tight joints.

In Fig. 11 is disclosed such a device incorporating my invention as applied to a mercury pool type of device having a metal container 150. It is desired to have an insulated lead-in for the anode 151 through an opening 152 in the metal casing. A porcelain tube 153 surrounds the anode lead 154 and has an extension 155 extending through the opening 152 of the metal casing. Another porcelain tube 156 surrounds the interior portion of the anode lead 154 and has a depression 157 into which the extension 155 of the outer porcelain piece fits. A metal portion 158 on the inner portion of the anode lead and a similar metal portion 159 on the exterior portion of the anode lead 154 tightly clamp the two porcelain sections 153 and 156 together about the opening 152 in the top cover 150 of the tube. This arrangement is assembled preferably by first spot welding the metal portion 159 in place on the anode lead 154, placing the other parts thereon and spot welding the metal part 158 while the parts are held tightly in position. A tubular section 160 surrounds the exterior portion of the porcelain tube 153. A similar construction may be utilized to support the make-alive 161. The metal joints of the casing will then be sweated together at such joints as 162, 163 and 164. After this is done, the pocket formed by the extensions 165 and 166 of the interior metal portion 159 and the exterior portion 160 extending above the surface of the porcelain tube 153 is then filled with a glass material 167 to provide a vacuum-tight seal across the upper surface of the porcelain. In case it is desired to increase the creepage distance between these two metal portions an insulator 168, which may have any desired shape such as the form of a ring having a reverse bend, is sealed into the glass 167.

Fig. 12 discloses another modification in which the porcelain section 171 is placed on lead-in 172 and enclosed in tubular shell 173. The porcelain section 170 is then placed on the lead-in and cemented in position to shell 173. The lead 172 preferably has raised or ring portions 174 upon which the two porcelain portions 170 and 171 clamp. The shell 173 preferably has the tapered flange 175 to maintain the lower porcelain section in position. The shell 173 is preferably of the

nickel cobalt iron alloy previously described and is copper sweated at 176 to the container wall 171. Thereafter, the upper portion 178 of the nickel-cobalt-iron shell is filled with a sealing glass material 179 to provide a vacuum-tight seal between the anode lead-in 172 and the shell portion 173 that forms an extension of the metal casing.

Fig. 13 illustrates a type of device in which the lead-in combines all the features of mechanical 10 clamping as well as the sealing of the metal, glass and porcelain. The metal container 180 has a tubular extension 181 welded or copper sweated thereto. The anode lead 182 is provided with a 15 ring 183 thereon. The tubular section 181 has a constricted portion 184 that preferably has a tapered portion 185 similar in contour with the bottom 186 of a porcelain ring 187. This insulator is placed around the lead-in 182 and the lead-in dropped in place after the porcelain is 20 coated with a glass sealing material. The lead-in construction is then heated and sealed together and the top porcelain ring 188 is put in place. While the structure is being heated, a tool is placed 25 on top of the tube 181 and spins or swages the upper portion 189 down over the top of the porcelain. It is then permitted to cool and the glaze hardens or sets. The top portion need not be glazed.

In Fig. 14 is disclosed another type of insulator 30 in which the tube 190 is sealed by means of glass 191 to the lower tubular tapered portion 192 of an elongated insulator 193. The upper tapered portion 194 of the insulator is closed with a cap 195 which has an exterior lead 196 and an interior lead 197 welded thereto. The insulator 193 preferably has extensions 198 to provide a greater 35 creepage distance between the metal portions 190 and 195.

I have previously described a preferred sealing 40 metal as being a nickel-cobalt-iron alloy and also the glass as being a boro-silicate type because these substances have a similar coefficient of expansion, substantially in the region of 4.6 to  $7.0 \times 10^{-6}$  cm. per degrees centigrade. I also desire 45 to utilize the ceramic material such as porcelain of a substantially similar coefficient of expansion. One such type of porcelain is composed of 30% feldspar, 25% flint and 45% clay. A typical chemical analysis of a particular type of this 50 porcelain known as "Derry plastic body" gives

|                                | Per cent |
|--------------------------------|----------|
| SiO <sub>2</sub>               | 70.97    |
| Al <sub>2</sub> O <sub>3</sub> | 23.15    |
| Fe <sub>2</sub> O <sub>3</sub> | 0.39     |
| TiO <sub>2</sub>               | 0.76     |
| CaO                            | 0.12     |
| MgO                            | 0.14     |
| Na <sub>2</sub> O              | 1.09     |
| K <sub>2</sub> O               | 3.30     |

In Fig. 15 I have shown curves disclosing the 60 unit expansion over a temperature range for these three materials.

The metals, porcelains and glasses do not necessarily have to have the same coefficient of expansion throughout the temperature range, but do have to have substantially the same coefficient of expansion in the annealing range of the glass as illustrated in Figs. 15 and 16. After the sealing has taken place, for example, in the temperature range 800° to 1100° C., the assembly is cooled to the annealing range of the glass and any stresses developed due to the difference of expansion as the different parts cool are then relieved because the glass, although set, is still

plastic enough to relieve stresses. The time required for this annealing will depend upon the exact type of glass, the temperature at which it is held and how closely the various materials match in the higher temperature range. This time will, 5 in general, be from a few minutes to four hours. The seal may then be rapidly cooled, and only care taken that improper cooling does not crack the porcelain.

The annealing range covers from the strain 10 point to the annealing point. The strain point is defined as that temperature at which practically all stresses (90% or better) are relieved in a period of four hours. The anneal point is defined as that temperature at which practically all 15 stresses are relieved in fifteen minutes.

The porcelains and glasses are of brittle type materials which are stronger in compression than tension. It is accordingly desirable that the metal should have a slightly higher unit expansion 20 in the annealing range so that, after the seals have been annealed and are cooled, the metal contracts slightly more than the porcelain and tends to clamp on the porcelain putting it slightly in compression.

Other types of porcelain with the desired coefficient of expansion may, of course, be substituted for this particular Derry plastic. Fig. 16 discloses a curve for such a body which I have designated as a "special Derry body" in which 30 pyrophyllite was substituted for the flint in the regular "Derry plastic body," together with curves for the preferred metal and glass in Fig. 15.

Although I have shown and described the invention applied to discharge tubes, many other 35 applications of my invention are possible. Such applications include bushing or lead-in for condensers, especially where such bushings must be oil or air-tight, electrical lead-in for hermetically-sealed refrigerators, lead-in bushings for sealed oil-filled transformers, lead-in for motors having a special cooling atmosphere as hydrogen, etc. This list is to be taken as illustrative and not as a limiting list.

My Patent No. 2,147,417 has claims covering 45 the seal of Fig. 5 herein, and my Patent No. 2,144,558 has claims covering Fig. 9 herein.

Also, although I have described various modifications of my invention, various changes may be made in the shape, arrangement, selection and application of the various elements and combinations disclosed. I accordingly desire only such 50 limitations to be placed on the following claims as is necessitated by the prior art.

I claim as my invention:

1. A terminal for a metallic enclosure comprising a porcelain member at least partially surrounded by a wall portion, said wall portion forming a part of said enclosure and having a surface adjacent said porcelain member comprising an alloy of 28% to 34% nickel, 5% to 25% cobalt, less than 1% manganese and the remainder substantially iron, the space between said porcelain and said surface being filled with a glass fused to said porcelain and to said alloy.

2. A terminal for a metallic enclosure, comprising a porcelain member at least partially surrounded by a wall portion, said wall portion forming a part of said enclosure and having a surface adjacent said porcelain member comprising an alloy of 28% to 34% nickel, 5% to 25% cobalt, less than 1% manganese and the remainder substantially iron, the space between said porcelain and said surface being filled with a boro-silicate glass fused to said porcelain and to said alloy.

3. A terminal for a metallic enclosure comprising a member of ceramic material at least partially surrounded by a wall portion, said wall portion forming a part of said enclosure and having a surface adjacent said member of ceramic material comprising an alloy of 28% to 34% nickel, 5% to 25% cobalt, less than 1% manganese and the remainder substantially iron, the space between said ceramic material and said surface being filled with a glass fused to said ceramic material and to said alloy.
4. A terminal for a metallic enclosure comprising a porcelain member at least partially surrounded by a wall portion, said wall portion forming a part of said enclosure and having a surface adjacent said porcelain member comprising an alloy of 28% to 34% nickel, 5% to 25% cobalt, less than 1% manganese and the remainder substantially iron, the space between said porcelain and said surface being filled with a glass fused to said porcelain and to said alloy, said porcelain member having a hole therethrough, a conductor extending through said hole and having at least its surface adjacent said
5. A terminal for a metallic enclosure comprising a porcelain member having a hole therethrough, a conductor having a surface comprising an alloy of 28% to 34% nickel, 5% to 25% cobalt, less than 1% manganese and the remainder substantially iron adjacent said porcelain member, and a layer of glass forming a fused junction to both said surface and said porcelain member.
6. A terminal for a metallic enclosure comprising a porcelain member having a hole therethrough, a conductor having a surface comprising an alloy of 28% to 34% nickel, 5% to 25% cobalt, less than 1% manganese and the remainder substantially iron adjacent said porcelain member, and a layer of boro-silicate glass forming a fused junction to both said surface and said porcelain member.

WALTER E. BAHLS.